

July 28, 1931.

A. B. RAY

1,816,125

SOLIDIFIED FUEL AND PROCESS OF MAKING THE SAME

Filed Nov. 29, 1927

*Fig. 1.*



*Fig. 2.*



*Fig. 3.*



Inventor  
Arthur B. Ray

By his Attorneys  
Hogans & Keary

## UNITED STATES PATENT OFFICE

ARTHUR B. RAY, OF BAYSIDE, NEW YORK

## SOLIDIFIED FUEL AND PROCESS OF MAKING THE SAME

Application filed November 29, 1927. Serial No. 236,392.

My invention relates to a solidified fuel containing a non-saponifiable combustible normally existing in the liquid state. In particular the invention relates to the production of solidified fuels in which the principal combustible constituent is alcohol or hydrocarbon liquids, such as gasoline, kerosene, benzene, etc., or a mixture of two or more of these combustible materials. 5

10 Solidified fuels of this general character which have heretofore been placed on the market have been characterized by the use as the solidifying agent of a base of nitrated cotton or pyroxylin in which alcohol or other combustible liquid is held. In order to insure against premature and undue liquefaction of the fuel during burning, it is necessary that the proportion of pyroxylin to alcohol be relatively large. Such fuels are 15

20 objectionable because of the fact that the pyroxylin in burning tends to flare or flash up and occasionally sparks are thrown from the burning mass for a considerable distance, thus giving rise to a very real fire hazard. 25

25 Also, as the alcohol-pyroxylin material is consumed, the height of the flame above the top of the can varies and the flame burns unsteadily or flickers because of the unsatisfactory air supply to the material burning deep 30

30 down in the container. This progressive lowering of the flame in the container is decidedly objectionable. It has been proposed to decrease the amount of pyroxylin required to keep the alcohol in a solidified condition 35

35 by substituting for a portion thereof cane pith or a similar non-fibrous cellulosic material. However, the cane pith alone will not absorb all of the alcohol required to form a satisfactory fuel and hold it in solidified form. Consequently the proportion of pyroxylin required, even when the cane pith is used, is sufficiently large to cause the objectionable burning characteristics of pyroxylin to be noticeable when the fuel is used. 40

45 It is an aim of my invention to produce a solidified fuel composed largely of alcohol or a hydrocarbon liquid which will burn smoothly and freely without sputtering or emission of sparks, which in burning does not liquefy prematurely or to an undue 45

degree and which permits the zone of combustion to be always maintained at or near the top of the container where air has ready access. A further object of my invention is to produce a solidified fuel unit which when ignited tends to burn with a steady, uniform localized flame, thus permitting of concentration of the heat evolved and the application thereof for useful purposes. 55

60 Other objects and advantages of the invention will appear as the description proceeds.

According to the present invention a highly absorbent, porous filler is incorporated with a mixture of a non-acidic, non-saponifiable, inflammable liquid and an alkali soap 65 of a heavy fatty acid, such for example as stearic or palmitic acid. The inflammable liquid is preferably solidified by the process described in my U. S. Patent No. 1,484,190, and it will be understood that the various 70 liquid fuels and the various modifications of the procedure for bringing about solidification therein disclosed may be applied in producing a solidified fuel according to the present invention. A combustible filler is preferred, although a highly inflammable material or one that tends to burn with explosive violence or to emit sparks is to be avoided. 75

80 The comminuted filler may be added to the liquid fuel before solidification or the liquid may be poured into containers in which the filler in comminuted or coherent form has been arranged or molded in a suitable manner. It is desirable that the filler hold together and so remain in position in the container after the solidified fuel has been partly consumed. Fibrous materials tend to form a coherent mat or mass which is further held together by residual framework of soap left behind as the fuel is consumed. In some 85 cases a small amount of a suitable binding material such as resin, gum, water glass etc. may be introduced to keep the filler in a satisfactory coherent mass. If desired, the filler may be held in position in the container 90 by means of a screen or other mechanical support. Because the filler has a very high porosity the reduction in amount of solidified fuel which can be placed in a container is 95 small. Furthermore it is not necessary nor, 100

usually desirable to distribute the filler throughout the entire mass of solidified liquid. I have found that particularly good results are obtained if the fuel is distributed in the container so that there are spaces filled only with the solidified fuel.

Preferred forms of my solidified fuel unit are illustrated in the accompanying drawings, in which:

- 10 Fig. 1 is a top plan view of a solidified fuel unit consisting of a central core of the solidified fuel unmixed with filler, such core being surrounded by additional solidified fuel mixed with an absorbent filler;
- 15 Fig. 2 is a vertical sectional view taken on the line 2—2 of Fig. 1; and

Fig. 3 is a top plan view of a modification in which instead of providing a single core centrally disposed in the filler mass, a plurality of cores or plugs of solidified fuel unmixed with filler are arranged at spaced distances in the solidified fuel-filler mass.

Referring more specifically to the drawings, 1 indicates a suitable metal container 25 and 2 a body of the solidified materials having substantially uniformly dispersed therethrough a suitable absorbent filler. In Figs. 1 and 2 a centrally-disposed core 3 of solidified fuel unmixed with filler is shown, where- 30 as in Fig. 3 a plurality of smaller plugs or zones 3a characterized by the absence of absorbent filler are provided.

As indicated above, it is preferred that a combustible but not a violently combustible 35 filler, be used. Materials which possess the desired absorbent and other properties above indicated are wood fibre, wood pulp, wood flour, cotton fibre, cane pith, corn stalk pith, dry peat, balsa wood, cellulose, bark, charcoal and 40 carbon. It will also be understood that certain non-combustible materials may be used advantageously. For some purposes and with some fuels such materials may be preferred. Examples of such materials which 45 may be used successfully are mineral wool and asbestos fibre. Of the non-combustible materials, mineral wool has been used with especially good results.

The combustion of the solidified fuel and 50 the filler, where a combustible filler is used, may be promoted, if desired, by impregnating the filler, or the fuel before incorporation therewith, with a suitable oxidizing agent or oxygen-containing compound, such for in- 55 stance as ammonium nitrate.

The type of material, its physical form, and method of placing in the container will be determined by the kind of solidified fuel, shape and size of container, and the manner 60 of using the fuel. A specific example may be described as follows:

Denatured alcohol is heated to approximately 70° C. and 3% of its weight of stearic acid is dissolved in it. Then approximately 65 the theoretical amount of sodium hydroxide

in a water-alcohol solution is added to form sodium stearate. After stirring for a few minutes to insure thorough mixing, the hot liquid is poured into suitable containers, for example, 8-oz. friction top cans, each containing approximately 1/2 oz. of comminuted cane pith. This amount of cane pith approximately fills the can but it has such high porosity and absorbent properties that its actual displacement volume is very small. When the mixture of liquid and filler cools a solid mass results which is an excellent solidified fuel. A solidified fuel unit having even more satisfactory burning properties is produced if a rod or similar member of approximately an 75 inch in diameter is placed in the middle of the can, either while the material is hot and before solidification or before the hot liquid fuel and soap solidifier are introduced, and maintained in position until the fuel is solidified, when it is removed and the hole which it leaves is filled with more hot liquid fuel and soap solidifier.

When the fuel unit is first ignited the core of solid fuel without filler vaporizes more 90 readily than the surrounding fuel with filler so the flame resulting from the combustion of the unit is concentrated in the region of the core. Any liquid formed during the combustion of the core of fuel without filler is immediately absorbed by the surrounding mass of porous filler. As the combustion of the unit proceeds the height of the core decreases and an increasingly large surface of the surrounding mass of fuel with filler is exposed. 100 Vaporization of the fuel is thus facilitated and since the larger part of the fuel is vaporized from the walls of the core space the flame resulting from the combustion of this vapor remains concentrated in the region of 105 the core space after the core has been consumed.

It will be understood that the porous filler not only absorbs any liquid which may be formed but that it also tends to act on the 110 principle of a wick to cause the alcohol or other liquid fuel, as the combustion proceeds, to move from the interior portions of the filler mass to the surface where combustion is taking place. Where it is desired to maintain the combustion zone at a level approximately that of the surface of the fuel when the container is completely filled before combustion is initiated, it may be desirable to use a non-combustible filler, in which case 115 combustion will continue near the top of the can and the fuel will be diffused to the exposed surface for combustion until the fuel is exhausted.

But even when a combustible filler is used the flame level is not materially lowered as long as the fuel is being freely vaporized from the surface of the filler. A slight lowering of the level will be caused by the charring and consequent shrinkage of cellu- 120

losic fillers but it is only after practically all the solidified fuel is exhausted that such fillers will be slowly burned. This slight lowering flame level when a combustible filler is used does not, however, interfere with the free burning of the fuel, particularly when a central zone or core of fuel unmixed with filler is provided.

The filler has the further advantage that it acts in some measure as an insulating material to prevent the rapid conduction of heat to the whole mass of fuel and to the bottom and walls of the container. Because of their higher heat value and lower cost, gasoline, kerosene, benzol or other liquid hydrocarbons are preferred in some cases. In these cases it will be understood that the formation of the stearate or other soap solidifier is preferably brought about by the use of a solution of caustic soda in a water-alcohol mixture, as described more particularly in my earlier patent above mentioned. It will also be understood that, instead of using substantially pure stearic acid, the commercial acid containing impurities up to 20%, such as palmitic acid, may be employed. Also while stearic acid is preferred, palmitic acid may be used if desired. Various modifications in the details of the procedure outlined and the proportions of the various constituents of the solidified fuel, as for example the filler, stearate or other soap solidifier, etc., may be resorted to without departing from the scope of the invention, which is not to be deemed as limited other than as indicated in the appended claims.

What I claim is:

1. A solidified fuel unit comprising a mass of solidified fuel having an absorbent filler uniformly distributed throughout certain portions thereof, and localized portions in which the fuel is unmixed with filler, said portions defining centralized areas of combustion.

2. A solidified fuel unit comprising a mass of solidified fuel having an absorbent filler uniformly distributed therethrough, and means for concentrating the flame during combustion of said fuel, said means comprising a body of solidified fuel unmixed with filler and disposed in operative relation to the said mass.

3. A solidified fuel unit comprising a container, an absorbent filler disposed within said container, a solidified fuel held by said filler, and means for localizing and centering the flame during combustion of said fuel to a limited portion of the exposed surface of the fuel in said container, said means comprising a core of solidified fuel unmixed with filler and extending from said exposed surface inwardly of the fuel mass.

4. Process of making a solidified fuel unit which comprises adding to a heated, non-acidic, non-saponifiable, organic liquid, a

small amount of a heavy fatty acid whose alkali soap is solid at ordinary temperatures, saponifying said acid by adding a solution of an alkali in water-alcohol mixture, intimately admixing the resulting mixture while hot 70 with an absorbent filler, and permitting the final admixture to cool.

5. Process of making a solidified fuel unit which comprises forming a mixture of a non-saponifiable combustible, organic liquid and 75 an alkali soap of a heavy fatty acid, bringing a portion of said mixture while heated to a fluid state into admixture with the mass of porous, absorbent filler material, defining openings in said mass and after the said mixture has solidified in said filler, filling said openings with additional solidified fuel unmixed with filler.

6. A solidified fuel unit comprising a container, an absorbent filler impregnated 85 with solidified fuel disposed therein, and a core of solidified fuel substantially free from filler.

7. A solidified fuel unit comprising a container, a fibrous absorbent filler impregnated 90 with solidified fuel disposed therein, and a core of solidified fuel substantially free from filler.

8. A solidified fuel unit comprising a substantially cylindrical container, an annular 95 mass of absorbent filler disposed therein and impregnated with solidified fuel, and a central core of solidified fuel substantially free from filler disposed within said annular mass of filler.

9. A solidified fuel unit comprising a substantially cylindrical container, an annular mass of absorbent, heat insulating, filler disposed therein adjacent the wall of said container and impregnated with solidified fuel, 105 and a central core of solidified fuel substantially free from filler disposed within said annular mass of filler.

10. A fuel unit comprising a container; a filler and solidified fuel, said filler being composed of a porous mass of coherent non-combustible fibres having at least one substantially fibre-free core-space therein, said solidified fuel being disposed in the container so as to fill said pores and core-space.

In testimony whereof, I have signed my name to this specification this 23d day of Nov., 1927.

ARTHUR B. RAY.

120

125

130